



US008454815B2

(12) **United States Patent**  
**Niazimbetova et al.**

(10) **Patent No.:** **US 8,454,815 B2**  
(45) **Date of Patent:** **\*Jun. 4, 2013**

(54) **PLATING BATH AND METHOD**

(75) Inventors: **Zuhra I. Niazimbetova**, Westborough, MA (US); **Maria Anna Rzeznik**, Shrewsbury, MA (US)

(73) Assignee: **Rohm and Haas Electronics Materials LLC**, Marlborough, MA (US)

(\*) Notice: Subject to any disclaimer, the term of this patent is extended or adjusted under 35 U.S.C. 154(b) by 0 days.

This patent is subject to a terminal disclaimer.

(21) Appl. No.: **13/280,135**

(22) Filed: **Oct. 24, 2011**

(65) **Prior Publication Data**

US 2013/0098770 A1 Apr. 25, 2013

(51) **Int. Cl.**

**C08G 59/14** (2006.01)  
**C09K 3/00** (2006.01)  
**C23C 18/38** (2006.01)  
**C25D 3/38** (2006.01)

(52) **U.S. Cl.**

USPC ..... **205/297**; 106/1.26; 252/183.11;  
528/118

(58) **Field of Classification Search**

None

See application file for complete search history.

(56) **References Cited**

**U.S. PATENT DOCUMENTS**

|                   |         |                                  |
|-------------------|---------|----------------------------------|
| 3,954,575 A       | 5/1976  | Yanagida et al.                  |
| 4,038,161 A       | 7/1977  | Eckles et al.                    |
| 4,169,772 A       | 10/1979 | Lowery et al.                    |
| 4,861,442 A       | 8/1989  | Tanaka et al.                    |
| 7,128,822 B2      | 10/2006 | Wang et al.                      |
| 8,262,895 B2 *    | 9/2012  | Niazimbetova et al. .... 205/297 |
| 8,268,157 B2 *    | 9/2012  | Niazimbetova ..... 205/297       |
| 8,268,158 B2 *    | 9/2012  | Niazimbetova et al. .... 205/297 |
| 2005/0045486 A1   | 3/2005  | Sahoda et al.                    |
| 2005/0045488 A1   | 3/2005  | Paneccasio et al.                |
| 2007/0007143 A1 * | 1/2007  | Hayashi et al. ..... 205/125     |
| 2010/0126872 A1 * | 5/2010  | Paneccasio et al. ..... 205/123  |
| 2011/0220512 A1   | 9/2011  | Niazimbetova et al.              |
| 2011/0220513 A1   | 9/2011  | Niazimbetova et al.              |
| 2011/0220514 A1   | 9/2011  | Niazimbetova                     |

\* cited by examiner

*Primary Examiner* — Robert Sellers

(74) *Attorney, Agent, or Firm* — S. Matthew Cairns

(57) **ABSTRACT**

Copper plating baths containing a leveling agent that is a reaction product of one or more of certain pyridine compounds with one or more epoxide-containing compounds, that deposit copper on the surface of a conductive layer are provided. Such plating baths deposit a copper layer that is substantially planar on a substrate surface across a range of electrolyte concentrations. Methods of depositing copper layers using such copper plating baths are also disclosed.

**12 Claims, No Drawings**

**1**  
**PLATING BATH AND METHOD**

The present invention relates generally to the field of electrolytic metal plating. In particular, the present invention relates to the field of electrolytic copper plating.

Methods for electroplating articles with metal coatings involve passing a current between two electrodes in a plating solution where one of the electrodes is the article to be plated. A typical copper plating bath comprises dissolved copper, an electrolyte in an amount sufficient to impart conductivity to the bath, and proprietary additives such as accelerators, leveling, and/or suppressors to improve the uniformity and quality of the copper deposit.

Electrolytic copper plating solutions are used in a variety of industrial applications, particularly for the fabrication of printed circuit boards ("PCBs") and semiconductors. For PCB fabrication, copper is electroplated over selected portions of the surface of a PCB, into blind vias and onto the walls of through-holes passing between the surfaces of the circuit board. The walls of a through-hole are first made conductive, such as by electroless metal deposition, before copper is electroplated onto the walls of the through-hole. Plated through-holes provide a conductive pathway from one board surface to another. For semiconductor fabrication, copper is electroplated over a surface of a wafer containing a variety of features such as vias, trenches or a combination thereof. The vias and trenches are metallized to provide conductivity between various layers of the semiconductor device.

Plating a substrate having irregular topography poses particular difficulties. During electroplating, a voltage drop variation typically exists along an irregular surface which can result in an uneven metal deposit, where a thicker metal deposit is observed over such surface irregularities. Leveling agents are often used in copper plating baths to provide substantially uniform, or level, copper layers in electronic devices. Recent approaches for high density interconnects have been developed which utilize blind vias. The desire is to maximize via filling while minimizing thickness variation in the copper deposit across the substrate surface. This is particularly challenging when the PCB contains both through-holes and blind vias.

U.S. Pat. No. 4,038,161 (Eckles et al.) discloses an acid copper electroplating bath which may include a reaction product of an epihalohydrin with a certain pyridine compound. The epihalohydrin may be epichlorohydrin or epibromohydrin. No other epoxide compounds are disclosed in this patent.

U.S. Pat. App. Pub. No. 2010/0126872 (Panecascio et al.) discloses acid copper electroplating baths containing a reaction product of a dipyridyl compound and an alkylating agent as a leveler compound. The alkylating agent may be an epoxide compound having a leaving group on a carbon alpha to the epoxy group. Suitable leaving groups are chloride, bromide, iodide, tosyl, triflate, sulfonate, mesylate, methosulfate, fluorosulfonate, methyl tosylate, brosylate or nosylate. The only exemplified epoxy compound alkylating agent is an alpha-leaving group substituted hydron, such as epihalohydrin.

Generally, leveling agents used in copper plating baths provide better leveling of the deposit across the substrate surface but tend to worsen the throwing power of the electroplating bath. Throwing power is defined as the ratio of the hole center copper deposit thickness to its thickness at the surface. Newer PCBs often contain both through-holes and blind vias. Conventional leveling agents, such as reaction products of pyridine with an alkylating agent epoxy compound such as epihalohydrin, do not provide sufficiently level

**2**

copper deposits on the substrate surface and fill through-holes and/or fill blind vias effectively. There remains a need in the art for leveling agents for copper electroplating baths used in the manufacture of electronic devices that provide sufficiently level copper deposits while maintaining sufficient throwing power of the bath to effectively fill apertures such as blind vias and through-holes.

The present invention provides a copper electroplating bath comprising: a source of copper ions; an electrolyte; and 10 a leveling agent comprising a reaction product of a pyridine compound of the formula (I)



wherein R<sup>1</sup>, R<sup>3</sup> and R<sup>5</sup> are independently chosen from H, (C<sub>1</sub>-C<sub>6</sub>)alkyl, Cy<sup>1</sup>, R<sup>6</sup>-Cy<sup>1</sup>, NR<sup>7</sup>R<sup>8</sup>, and R<sup>6</sup>-NR<sup>7</sup>R<sup>8</sup>; Cy<sup>1</sup> is a 5- to 6-membered ring; R<sup>2</sup> and R<sup>4</sup> are independently chosen from H, (C<sub>1</sub>-C<sub>6</sub>)alkyl, and (C<sub>6</sub>-C<sub>12</sub>)aryl; R<sup>2</sup> may be taken together with R<sup>1</sup> or R<sup>3</sup> along with the atoms to which they are attached to form a fused 5- to 6-membered ring; R<sup>4</sup> may be taken together with R<sup>3</sup> or R<sup>5</sup> along with the atoms to which they are attached to form a fused 5- to 6-membered ring; R<sup>6</sup> is a (C<sub>1</sub>-C<sub>10</sub>)hydrocarbyl group; R<sup>7</sup> and R<sup>8</sup> are independently chosen from H, (C<sub>1</sub>-C<sub>6</sub>)alkyl, (C<sub>6</sub>-C<sub>10</sub>)aryl, (C<sub>1</sub>-C<sub>6</sub>)alkyl(C<sub>6</sub>-C<sub>10</sub>)aryl, and (C<sub>2</sub>-C<sub>6</sub>)alkenyl(C<sub>6</sub>-C<sub>10</sub>)aryl; R<sup>7</sup> and R<sup>8</sup> may be taken together to form a 5- or 6-membered heterocyclic ring; and R<sup>7</sup> and R<sup>8</sup> may be taken together along with the atoms to which they are attached to form a 5- to 6-membered fused nitrogen-containing ring, with an epoxide-containing compound; provided that at least one of R<sup>1</sup>, R<sup>3</sup> and R<sup>5</sup> is NR<sup>7</sup>R<sup>8</sup> when the epoxide-containing compound has a leaving group on a carbon alpha to an epoxide group.

The present invention further provides a method of depositing copper on a substrate comprising: contacting a substrate to be plated with the copper electroplating bath described above; and applying a current density for a period of time sufficient to deposit a copper layer on the substrate.

Also provided by the present invention is a reaction product of one or more pyridine compounds with one or more epoxide-containing compounds; wherein the pyridine compound has the formula (I)



wherein R<sup>1</sup>, R<sup>3</sup> and R<sup>5</sup> are independently chosen from H, (C<sub>1</sub>-C<sub>6</sub>)alkyl, Cy<sup>1</sup>, R<sup>6</sup>-Cy<sup>1</sup>, NR<sup>7</sup>R<sup>8</sup>, and R<sup>6</sup>-NR<sup>7</sup>R<sup>8</sup>; Cy<sup>1</sup> is a 5- to 6-membered ring; R<sup>2</sup> and R<sup>4</sup> are independently chosen from H, (C<sub>1</sub>-C<sub>6</sub>)alkyl, and (C<sub>6</sub>-C<sub>12</sub>)aryl; R<sup>2</sup> may be taken together with R<sup>1</sup> or R<sup>3</sup> along with the atoms to which they are attached to form a fused 5- to 6-membered ring; R<sup>4</sup> may be taken together with R<sup>3</sup> or R<sup>5</sup> along with the atoms to which they are attached to form a fused 5- to 6-membered ring; R<sup>6</sup> is a (C<sub>1</sub>-C<sub>10</sub>)hydrocarbyl group; R<sup>7</sup> and R<sup>8</sup> are independently

chosen from H, (C<sub>1</sub>-C<sub>6</sub>)alkyl, (C<sub>6</sub>-C<sub>10</sub>)aryl, (C<sub>1</sub>-C<sub>6</sub>)alkyl(C<sub>6</sub>-C<sub>10</sub>)aryl, and (C<sub>2</sub>-C<sub>6</sub>)alkenyl(C<sub>6</sub>-C<sub>10</sub>)aryl; R<sup>7</sup> and R<sup>8</sup> may be taken together to form a 5- or 6-membered heterocyclic ring; and R<sup>7</sup> and R<sup>4</sup> may be taken together along with the atoms to which they are attached to form a 5- to 6-membered fused nitrogen-containing ring; and wherein at least one epoxide-containing compound has the formula



where Y, Y<sup>1</sup> and Y<sup>2</sup> are independently chosen from H and (C<sub>1</sub>-C<sub>4</sub>)alkyl; each Y<sup>3</sup> is independently chosen from H, an epoxy group, and (C<sub>1</sub>-C<sub>5</sub>)alkyl; X=CH<sub>2</sub>X<sup>2</sup> or (C<sub>2</sub>-C<sub>6</sub>)alkenyl; X<sup>1</sup>=H or (C<sub>1</sub>-C<sub>5</sub>)alkyl; X<sup>2</sup>=halogen, O(C<sub>1</sub>-C<sub>3</sub>)alkyl or O(C<sub>1</sub>-C<sub>3</sub>)haloalkyl; A=OR<sup>11</sup> or R<sup>12</sup>; R<sup>11</sup>=((CR<sup>13</sup>R<sup>14</sup>)<sub>m</sub>O)<sub>n</sub>, (aryl-O)<sub>p</sub>, CR<sup>13</sup>R<sup>14</sup>-Z-CR<sup>13</sup>R<sup>14</sup>O or OZ<sup>1</sup>, O; R<sup>12</sup>=(CH<sub>2</sub>)<sub>y</sub>; A<sup>1</sup> is a (C<sub>5</sub>-C<sub>12</sub>)cycloalkyl ring or a 5- to 6-membered cyclic sulfone ring; Z=a 5- or 6-membered ring; Z<sup>1</sup> is R<sup>15</sup>OArOR<sup>15</sup>, (R<sup>16</sup>O)<sub>a</sub>Ar(OR<sup>16</sup>)<sub>a</sub>, or (R<sup>16</sup>O)<sub>a</sub>Cy<sup>2</sup>(OR<sup>16</sup>)<sub>a</sub>; Z<sup>2</sup>=SO<sub>2</sub> or



Cy<sup>2</sup>=(C<sub>5</sub>-C<sub>12</sub>)cycloalkyl; each R<sup>13</sup> and R<sup>14</sup> are independently chosen from H, CH<sub>3</sub> and OH; each R<sup>15</sup> represents (C<sub>1</sub>-C<sub>8</sub>)alkyl; each R<sup>16</sup> represents a (C<sub>2</sub>-C<sub>6</sub>)alkyleneoxy; each a=1-10; m=1-6; n=1-20; p=1-6; q=1-6; r=0-4; t=1-4; v=0-3; and y=0-6; wherein Y<sup>1</sup> and Y<sup>2</sup> may be taken together to form a (C<sub>8</sub>-C<sub>12</sub>)cyclic compound; provided that at least one of R<sup>1</sup>, R<sup>3</sup> and R<sup>5</sup> is NR<sup>7</sup>R<sup>8</sup> when the epoxide-containing compound has the formula (E-I), X=CH<sub>2</sub>X<sup>2</sup> and X<sup>2</sup>=halogen.

As used throughout this specification, the following abbreviations shall have the following meanings, unless the context clearly indicates otherwise: A/dm<sup>2</sup>=amperes per square decimeter; ° C.=degrees Celsius; g=gram; mg=milligram; L=liter; ppm=parts per million; μm=micrometer; mm=millimeters; cm=centimeters; DI=deionized; mmol=millimoles; and mL=milliliter. All amounts are percent by weight and all ratios are molar ratios, unless otherwise noted. All numerical ranges are inclusive and combinable in any order, except where it is clear that such numerical ranges are constrained to add up to 100%.

As used throughout the specification, "feature" refers to geometries on a substrate. "Apertures" refer to recessed features including through-holes, blind vias and trenches. As used throughout this specification, the term "plating" refers to electroplating. "Deposition" and "plating" are used interchangeably. "Halide" refers to fluoride, chloride, bromide

and iodide. The term "alkyl" includes linear, branched and cyclic alkyl. "Alkenyl" includes linear, branched and cyclic alkenyl. "Accelerator" refers to an organic additive that increases the plating rate of the electroplating bath. A "suppressor" refers to an organic additive that suppresses the plating rate. "Leveler" refers to an organic compound that is capable of providing a substantially level (or uniform) metal layer. The terms "leveler" and "leveling agent" are used interchangeably throughout this specification. "Printed circuit boards" and "printed wiring boards" are used interchangeably herein. The articles "a" and "an" refer to the singular and the plural.

The copper plating baths of the present invention comprise a source of copper ions, an electrolyte, and a leveling agent that comprises a reaction product of one or more of certain pyridine compounds with one or more epoxide-containing compounds. The copper plating baths may additionally comprise one or more other additives such as halide ion, accelerators, suppressors, or additional leveling agents. The plating bath and method of the present invention are useful in providing a substantially level copper layer plated on a substrate, such as a printed circuit board or semiconductor substrate. Also, the present invention is useful in filling apertures in a substrate with copper. Such filled apertures are substantially free of voids. Copper deposits from the present invention are substantially free of nodules, that is, they have  $\leq 15$  nodules/95 cm<sup>2</sup> of surface area, and preferably  $<10$  nodules/95 cm<sup>2</sup>.

Any copper ion source that is at least partially soluble, and preferably soluble, in the electroplating bath is suitable. Suitable copper ion sources are copper salts and include without limitation: copper sulfate; copper halides such as copper chloride; copper acetate; copper nitrate; copper fluoroborate; copper alkylsulfonates; copper arylsulfonates; copper sulfamate; and copper gluconate. Exemplary copper alkylsulfonates include copper (C<sub>1</sub>-C<sub>6</sub>)alkylsulfonate and more preferably copper (C<sub>1</sub>-C<sub>3</sub>)alkylsulfonate. Preferred copper alkylsulfonates are copper methanesulfonate, copper ethanesulfonate and copper propanesulfonate. Exemplary copper arylsulfonates include, without limitation, copper phenyl sulfonate, copper phenol sulfonate and copper p-toluene sulfonate. Copper sulfate pentahydrate and copper methanesulfonate are preferred. Mixtures of copper ion sources may be used. Such copper salts are generally commercially available and may be used without further purification. The copper salts may be used in the present plating baths in any amount that provides sufficient copper ion concentration for electroplating copper on a substrate. Typically, the copper salt is present in an amount sufficient to provide an amount of copper (as metal or ions) of 10 to 180 g/L in the plating solution.

It will be appreciated that one or more soluble salts of metal ions other than copper ions may be advantageously added to the present electroplating baths when the deposition of copper alloys is desired. Alloys, such as copper-tin having up to 2% by weight tin, may be advantageously deposited according to the present invention. Other suitable copper alloys include, without limitation, copper-silver, tin-copper-silver, and tin-copper-bismuth. The amount of each of the metal salts in such mixtures depends upon the particular alloy to be plated and is well known to those skilled in the art.

The electrolyte useful in the present invention may be alkaline or acidic, and is preferably acidic. Suitable acid electrolytes include, but are not limited to, sulfuric acid, acetic acid, fluoroboric acid, alkanesulfonic acids such as methanesulfonic acid, ethanesulfonic acid, propanesulfonic acid and trifluoromethane sulfonic acid, arylsulfonic acids such as phenyl sulfonic acid, phenol sulfonic acid and toluene sul-

fonic acid, sulfamic acid, hydrochloric acid, and phosphoric acid. Mixtures of acids may be advantageously used. Preferred acids are sulfuric acid, methanesulfonic acid, ethanesulfonic acid, propanesulfonic acid, and mixtures thereof. The acids are typically present in an amount in the range of from 1 to 300 g/L, preferably from 5 to 250 g/L, and more preferably from 10 to 225 g/L. Electrolytes are commercially available from a variety of sources and may be used without further purification.

The reaction products used as leveling agents in the present invention contain at least one pyridine compound of the formula (I)



(I)

wherein R<sup>1</sup>, R<sup>3</sup> and R<sup>5</sup> are independently chosen from H, (C<sub>1</sub>-C<sub>6</sub>)alkyl, Cy<sup>1</sup>, R<sup>6</sup>-Cy<sup>1</sup>, NR<sup>7</sup>R<sup>8</sup>, and R<sup>6</sup>-NR<sup>7</sup>R<sup>8</sup>; Cy<sup>1</sup> is a 5- to 6-membered ring; R<sup>2</sup> and R<sup>4</sup> are independently chosen from H, (C<sub>1</sub>-C<sub>6</sub>)alkyl, and (C<sub>6</sub>-C<sub>12</sub>)aryl; R<sup>2</sup> may be taken together with R<sup>1</sup> or R<sup>3</sup> along with the atoms to which they are attached to form a fused 5- to 6-membered ring; R<sup>4</sup> may be taken together with R<sup>3</sup> or R<sup>5</sup> along with the atoms to which they are attached to form a fused 5- to 6-membered ring; R<sup>6</sup> is a (C<sub>1</sub>-C<sub>10</sub>)hydrocarbyl group; R<sup>7</sup> and R<sup>8</sup> are independently chosen from H, (C<sub>1</sub>-C<sub>6</sub>)alkyl, (C<sub>6</sub>-C<sub>10</sub>)aryl, (C<sub>1</sub>-C<sub>6</sub>)alkyl(C<sub>6</sub>-C<sub>10</sub>)aryl, and (C<sub>2</sub>-C<sub>6</sub>)alkenyl(C<sub>6</sub>-C<sub>10</sub>)aryl; R<sup>7</sup> and R<sup>8</sup> may be taken together to form a 5- or 6-membered heterocyclic ring; and R<sup>7</sup> and R<sup>4</sup> may be taken together along with the atoms to which they are attached to form a 5- to 6-membered fused nitrogen-containing ring. Preferably, R<sup>1</sup>, R<sup>3</sup> and R<sup>5</sup> are independently chosen from H, Cy<sup>2</sup>, R<sup>6</sup>-Cy<sup>1</sup>, NR<sup>7</sup>R<sup>8</sup>, and R<sup>6</sup>-NR<sup>7</sup>R<sup>8</sup>, and more preferably R<sup>1</sup>, R<sup>3</sup> and R<sup>5</sup> are independently chosen from H, Cy<sup>2</sup>, R<sup>6</sup>-Cy<sup>1</sup>, and NR<sup>7</sup>R<sup>8</sup>. It is more preferred that at least one of R<sup>1</sup>, R<sup>3</sup> and R<sup>5</sup> is not H, and more preferably that at least one of R<sup>1</sup>, R<sup>3</sup> and R<sup>5</sup> is independently chosen from Cy<sup>1</sup>, R<sup>6</sup>-Cy<sup>1</sup>, and NR<sup>7</sup>R<sup>8</sup>. When any of R<sup>1</sup>, R<sup>3</sup> and R<sup>5</sup> are independently (C<sub>1</sub>-C<sub>6</sub>)alkyl, it is preferred that such group is a (C<sub>1</sub>-C<sub>3</sub>)alkyl. Cy<sup>1</sup> may be any 5- to 6-membered ring, including carbocyclic and heterocyclic rings, which may be saturated, unsaturated or aromatic. It is preferred that R<sup>2</sup> and R<sup>4</sup> are independently chosen from H, (C<sub>1</sub>-C<sub>3</sub>)alkyl, and (C<sub>6</sub>-C<sub>10</sub>)aryl, and more preferably H, methyl, ethyl, propyl, phenyl, benzyl, and phenethyl, and most preferably H. The (C<sub>1</sub>-C<sub>12</sub>)hydrocarbyl group of R<sup>6</sup> may be (C<sub>1</sub>-C<sub>10</sub>)alkylene, (C<sub>2</sub>-C<sub>10</sub>)alkenylene, (C<sub>2</sub>-C<sub>10</sub>)alkynylene, (C<sub>6</sub>-C<sub>10</sub>)arylene, and (C<sub>1</sub>-C<sub>4</sub>)alkenylene(C<sub>6</sub>-C<sub>10</sub>)arylene. Preferably, R<sup>6</sup> is chosen from (C<sub>1</sub>-C<sub>6</sub>)alkylene, (C<sub>2</sub>-C<sub>6</sub>)alkenylene, phenylene, and —CH<sub>2</sub>C<sub>6</sub>H<sub>4</sub>—CH<sub>2</sub>—, and more preferably from (C<sub>1</sub>-C<sub>4</sub>)alkylene and (C<sub>2</sub>-C<sub>4</sub>)alkenylene, and still more preferably from —CH<sub>2</sub>—, —CH<sub>2</sub>CH<sub>2</sub>—, —(CH<sub>2</sub>)<sub>3</sub>—, —(CH<sub>2</sub>)<sub>4</sub>—, —(CH=CH)—, and —(CH<sub>2</sub>—CH=CH—CH<sub>2</sub>)—. R<sup>7</sup> and R<sup>8</sup> are preferably independently chosen from H, (C<sub>1</sub>-C<sub>3</sub>)alkyl, (C<sub>6</sub>-C<sub>10</sub>)aryl, (C<sub>1</sub>-C<sub>6</sub>)alkyl(C<sub>6</sub>-C<sub>10</sub>)aryl, and (C<sub>2</sub>-C<sub>6</sub>)alkenyl(C<sub>6</sub>-C<sub>10</sub>)aryl, more preferably H, (C<sub>1</sub>-C<sub>3</sub>)alkyl, phenyl, benzyl and phenethyl, and even more preferably H, methyl, ethyl, phenyl and benzyl. It is more preferred that at least one of R<sup>7</sup> and R<sup>8</sup> is not H, and even more preferred that both R<sup>7</sup> and R<sup>8</sup> are not H. Any of R<sup>1</sup>-R<sup>8</sup> may optionally be substituted by one or more groups chosen from hydroxyl, (C<sub>1</sub>-C<sub>6</sub>)alkoxy, and keto. By "substituted", it

is meant that 1 or more hydrogen atoms are replaced with one or more substituent group. In the case of a keto group, 2 hydrogens are replaced with 1 oxygen.

Exemplary Cy<sup>1</sup> groups include morpholine, piperidine, pyrrolidine, pyridine, imidazole, pyrrole, pyrazine, cyclopentane, cyclohexane, cyclopentene, and cyclohexene. Preferred Cy<sup>1</sup> groups include morpholine, piperidine, pyrrolidine, pyridine, and imidazole, more preferably morpholine, piperidine, pyrrolidine, and pyridine, and most preferably morpholine, 10 piperidine, and pyrrolidine.

When R<sup>2</sup> is taken together with R<sup>1</sup> or R<sup>3</sup> along with the atoms to which they are attached, and/or R<sup>4</sup> is taken together with R<sup>3</sup> or R<sup>5</sup> along with the atoms to which they are attached, to form a fused 5- to 6-membered ring, such fused ring may be 15 saturated, unsaturated, heterocyclic, or aromatic. Such fused ring may optionally be substituted, such as with hydroxyl, (C<sub>1</sub>-C<sub>6</sub>)alkyl, (C<sub>1</sub>-C<sub>6</sub>)alkoxy, amino, (C<sub>1</sub>-C<sub>6</sub>)alkylamino and di(C<sub>1</sub>-C<sub>6</sub>)alkylamino. Such fused ring may also be fused to one or more other rings, which may be saturated, unsaturated 20 or aromatic. Exemplary pyridine compounds having such fused rings include: 2H-pyrido[3,2-b][1,4]oxazin-3(4H)-one; quinoline; isoquinoline; 4-aminoquinoline; 4-(dimethylamino)-quinoline; 2-(dimethylamino)quinoline; 2-methylquinolin-4-amine; 1,10-phenanthroline; 1,5-naphthyridine; 1,8-naphthyridine; 2,8-dimethylquinoline; and 2-(2-pyridyl)quinoline.

When R<sup>7</sup> and R<sup>8</sup> may be taken together to form a 5- or 6-membered heterocyclic ring, such heterocyclic ring may be 30 saturated, unsaturated or aromatic. Such heterocyclic ring contains at least 1 nitrogen atom, and may contain 1 or more heteroatoms such as oxygen or sulfur. Preferably, such heterocyclic ring contains nitrogen and/or oxygen as the only heteroatoms. Such heterocyclic ring may optionally be substituted, such as with hydroxyl, (C<sub>1</sub>-C<sub>6</sub>)alkyl, (C<sub>1</sub>-C<sub>6</sub>)alkoxy, amino, (C<sub>1</sub>-C<sub>6</sub>)alkylamino and di(C<sub>1</sub>-C<sub>6</sub>)alkylamino. Exemplary heterocyclic rings include pyridine, piperidine, morpholine, and pyrrolidine.

Preferred pyridine compounds are: 2-aminopyridine; 4-aminopyridine; 2-(dimethylamino)pyridine; 4-(dimethylamino)pyridine; 2-(diethylamino)pyridine; 4-(diethylamino)pyridine; 2-(benzylamino)pyridine; quinoline; isoquinoline; 4-aminoquinoline; 4-(dimethylamino)quinoline; 2-(dimethylamino)quinoline; 2-methylquinolin-4-amine; 1,10-phenanthroline; 1,5-naphthyridine; 1,8-naphthyridine; 2,2'-dipyridylamine; 2,2'-bipyridine; 4,4'-bipyridine; 2,3-di-45 2-pyridyl-2,3-butanediol; di-2-pyridyl ketone; 2-(piperidin-1-yl)pyridine; 4-(pyridine-2-yl)morpholine; 4-(pyridine-4-yl)morpholine; 4-(pyrrolidin-1-yl)pyridine; 6-methyl-2,2'-bipyridine; 1,2-di(pyridine-4-yl)ethane; 1,3-di(pyridine-4-yl)propane; 1,2-di(pyridine-4-yl)ethene; 1,2-di(pyridine-2-yl)ethene; 2-(2-(pyridin-4-yl)vinyl)pyridine; 2H-pyrido[3,2-b][1,4]oxazin-3(4H)-one; 2-(2-methylaminoethyl)pyridine; 4-(ethylaminomethyl)-pyridine; N,N,2-trimethylpyridin-4-amine; 2,8-dimethylquinoline; and 2-(2-pyridyl)quinoline.

The pyridine compounds useful in the present invention are generally commercially available from a variety of sources, such as Sigma-Aldrich (St. Louis, Mo.) or may be prepared from literature methods. These compounds may be used as-is, or may be purified before being reacted with the one or more epoxy-containing compounds.

Any suitable epoxide-containing compound may be used to make the reaction products of the present invention, provided that when the epoxide-containing compound has a leaving group on a carbon alpha to an epoxide group that at least one of R<sup>1</sup>, R<sup>3</sup> and R<sup>5</sup> in formula (I) is NR<sup>7</sup>R<sup>8</sup>. A "carbon alpha to an epoxide group" refers to a carbon atom bonded to one of the epoxide carbons. Such leaving groups are chloride,

bromide, iodide, tosyl, triflate, sulfonate, mesylate, methosulfate, fluorosulfonate, methyl tosylate, brosylate and nosylate. Preferably, the epoxide-containing compound is free of a leaving group on each carbon alpha to each epoxide group. The present epoxide-containing compounds may contain 1 or more epoxide groups, and typically contain 1, 2 or 3 epoxide groups, and preferably contain 1 or 2 epoxide groups, and more preferably 2 epoxide groups. Suitable epoxide-containing compounds useful in the present invention are those of the formulae E-I, E-II, or E-III



where Y, Y<sup>1</sup> and Y<sup>2</sup> are independently chosen from H and (C<sub>1</sub>-C<sub>4</sub>)alkyl; each Y<sup>3</sup> is independently chosen from H, an epoxy group, and (C<sub>1</sub>-C<sub>6</sub>)alkyl; X=CH<sub>2</sub>X<sup>2</sup> or (C<sub>2</sub>-C<sub>6</sub>)alkenyl; X<sup>1</sup>=H or (C<sub>1</sub>-C<sub>5</sub>)alkyl; X<sup>2</sup>=halogen, O(C<sub>1</sub>-C<sub>3</sub>)alkyl or O(C<sub>1</sub>-C<sub>3</sub>)haloalkyl; A=OR<sup>11</sup> or R<sup>12</sup>; R<sup>1</sup>=(CR<sup>13</sup>R<sup>14</sup>)<sub>n</sub>, (aryl-O)<sub>p</sub>, CR<sup>13</sup>R<sup>14</sup>-Z-CR<sup>13</sup>R<sup>14</sup>O or OZ<sup>1</sup>O; R<sup>12</sup>=(CH<sub>2</sub>)<sub>y</sub>; A1 is a (C<sub>5</sub>-C<sub>12</sub>)cycloalkyl ring or a 5- to 6-membered cyclic-sulfone ring; Z=a 5- or 6-membered ring; Z<sup>1</sup> is R<sup>15</sup>OArOR<sup>15</sup>, (R<sup>16</sup>O)<sub>a</sub>Ar(OR<sup>16</sup>)<sub>a</sub>, or (R<sup>16</sup>O)<sub>a</sub>Cy<sup>2</sup>(OR<sup>16</sup>)<sub>a</sub>; Z<sup>2</sup>=SO<sub>2</sub> or



$Cy^2 = (C_5-C_{12})cycloalkyl$ ; each  $R^{13}$  and  $R^{14}$  are independently chosen from H,  $CH_3$  and OH; each  $R^{15}$  represents  $(C_1-C_8)alkyl$ ; each  $R^{16}$  represents a  $(C_2-C_6)alkyleneoxy$ ; each  $a=1-10$ ;  $m=1-6$ ;  $n=1-20$ ;  $p=1-6$ ;  $q=1-6$ ;  $r=0-4$ ;  $t=1-4$ ;  $v=0-3$ ; and  $y=0-6$ ; wherein  $Y^1$  and  $Y^2$  may be taken together to form a  $(C_8-C_{12})cyclic$  compound. Preferably  $Y=H$ . More preferably  $X^1=H$ . It is preferred that  $X=CH_2X^2$ . It is further preferred that  $X^2=halogen$  or  $O(C_1-C_3)fluoroalkyl$ . Even more preferred are compounds of formula E-I where  $Y=X^1=H$ ,  $X=CH_2X^2$  and  $X^2=O(C_1-C_3)alkyl$ .  $Y^1$  and  $Y^2$  are preferably independently chosen from H and  $(C_1-C_2)alkyl$ . When  $Y^1$  and  $Y^2$  are not joined to form a cyclic compound, it is preferred that  $Y^1$  and  $Y^2$  are both H. When  $Y^1$  and  $Y^2$  are joined to form a cyclic compound, it is preferred that A is  $R^{12}$  or a chemical bond and that a  $(C_8-C_{10})carbocyclic$  ring is formed. It is preferred that  $m=2-4$ . Preferably,  $n=1-10$ . It is further preferred that  $m=2-4$  when  $n=1-10$ . Phenyl-0 is the preferred aryl-O group for  $R^{11}$ . It is preferred that  $p=1-4$ , more preferably 1-3, and still more preferably 1-2. Z is preferably a 5- or 6-membered carbocyclic ring and, more preferably, Z is a 6-membered carbocyclic ring. Preferably,  $Z^2$  is

It is preferred that  $v=0-2$ . Preferably,  $y=0-4$ , and more preferably 1-4. When  $A=R^{12}$  and  $y=0$ , then  $A$  is a chemical bond. Preferably,  $m=1-6$ , and more preferably 1-4. It is preferred that  $q=1-4$ , more preferably 1-3, and still more preferably 1-2. Preferably,  $r=0$  and  $q=1$ , and more preferably  $Y^1$  and  $Y^2=H$ ,  $r=0$  and  $q=1$ . Preferably,  $Z^1=R^{15}OArOR^{15}$  or  $(R^{16}O)_aAr(OR^{16})_a$ . Each  $R^{15}$  is preferably  $(C_1-C_6)alkyl$  and more preferably  $(C_1-C_4)alkyl$ . Each  $R^{16}$  is preferably  $(C_2-C_4)alkyle-neoxy$ . It is preferred that  $t=1-2$ . Preferably,  $a=1-8$ , more preferably 1-6 and still more preferably 1-4. When  $Z^2$  is



it is preferred that A1 is a 6- to 10-membered carbocyclic ring, and more preferably a 6- to 8-membered carbocyclic ring.

Exemplary epoxide-containing compounds of formula E-1 include, without limitation, epihalohydrin, 1,2-epoxy-5-hexene, 2-methyl-2-vinyloxirane, and glycidyl 1,1,2,2-tetrafluoroethyl ether. Preferably, the epoxide-containing compound is epichlorohydrin or epibromohydrin, and more preferably epichlorohydrin.

30 Suitable compounds of formula E-II where  $R^{11} = ((CR^{13}R^{14})_mO)_n$  are those of the formula:



40 where  $Y^1$ ,  $Y^2$ ,  $R^{12}$ ,  $R^{13}$ ,  $R^{14}$ , n and m are as defined above. Preferably,  $Y^1$  and  $Y^2$  are both H. When m=2, it is preferred that each  $R^{13}$  is H,  $R^{14}$  is chosen from H and  $CH_3$ , and n=1-10. When m=3, it is preferred that at least one  $R^{14}$  is chosen from  $CH_3$  and OH, and n=1. When m=4, it is preferred that both  $R^{13}$  and  $R^{14}$  are H, and n=1. Exemplary compounds of formula E-IIa include, but are not limited to: 1,4-butanediol diglycidyl ether, ethylene glycol diglycidyl ether, di(ethylene glycol) diglycidyl ether, poly(ethylene glycol)diglycidyl ether compounds, glycerol diglycidyl ether, neopentyl glycol diglycidyl ether, propylene glycol diglycidyl ether, di(propylene glycol)diglycidyl ether, and poly(propylene glycol)diglycidyl ether compounds. Poly(ethylene glycol)diglycidyl ether compounds of formula E-IIa are those compounds where each of  $R^{13}$  and  $R^{14}$ =H, m=2, and n=3-20, and preferably n=3-15, more preferably n=3-12, and still more preferably n=3-10. Exemplary poly(ethylene glycol)diglycidyl ether compounds include tri(ethylene glycol)diglycidyl ether, tetra(ethylene glycol)diglycidyl ether, penta(ethylene glycol)diglycidyl ether, hexa(ethylene glycol)diglycidyl ether, nona(ethylene glycol)diglycidyl ether, deca(ethylene glycol)diglycidyl ether, and dodeca(ethylene glycol)diglycidyl ether. Poly(propylene glycol)diglycidyl ether compounds of formula E-IIa are those compounds where each of  $R^{13}$ =H and one of  $R^{14}$ = $CH_3$ , m=2, and n=3-20, and preferably n=3-15, more preferably n=3-12, and still more preferably n=3-10. Exemplary poly(propylene glycol)diglycidyl ether compounds include tri(propylene glycol)diglycidyl ether, tetra-

(propylene glycol)diglycidyl ether, penta(propylene glycol)diglycidyl ether, hexa(propylene glycol)diglycidyl ether, nona(propylene glycol)diglycidyl ether, deca(propylene glycol)diglycidyl ether, and dodeca(propylene glycol)diglycidyl ether. Suitable poly(ethylene glycol)diglycidyl ether compounds and poly(propylene glycol)diglycidyl ether compounds are those having a number average molecular weight of from 200 to 10000, and preferably from 350 to 8000.

Suitable compounds of formula E-II where  $R^{11}=(\text{aryl}-\text{O})_p$  are those having the formula E-IIb, E-IIc or E-IId:

(E-IIb)



(E-IIb)



(E-IIc) 20



30

(E-IId)

10 where  $Y^1$ ,  $Y^2$ ,  $R^{13}$  and  $R^{14}$  are as defined above, and  $q=0$  or 1. When  $q=0$ , the ring structure is a 5-membered carbocyclic ring and when  $q=1$ , the ring structure is a 6-membered carbocyclic ring. Preferably,  $Y^1$  and  $Y^2=H$ . More preferably,  $Y^1$  and  $Y^2=H$  and  $q=1$ . Preferred compounds of formula E-II where  $R^{11}=\text{CR}^{13}\text{R}^{14}-\text{Z}-\text{CR}^{13}\text{R}^{14}\text{O}$  are 1,2-cyclohexanediol diglycidyl ether and 1,4-cyclohexanediol diglycidyl ether.

15 When  $A=R^{12}$ , suitable compounds of formula E-II are those having the formula:



(E-IIe)

25 where  $Y^1$ ,  $Y^2$  and  $y$  are as defined above. It is preferred that  $y=0-4$ , more preferably  $y=1-4$ , and  $y=2-4$ . Exemplary compounds of formula E-IIe include, without limitation: 1,2,5,6-diepoxyhexane; 1,2,7,8-diepoxyoctane; and 1,2,9,10-diepoxydecane.

30 In compounds of formula II where  $A=\text{OZ}^1\text{O}$ , preferred compounds are those of the formula

(E-IIf)



50 where  $Y^1$ ,  $Y^2$  and  $p$  are as defined above, and each  $R^{17}$  represents  $(\text{C}_1-\text{C}_4)\text{alkyl}$  or  $(\text{C}_1-\text{C}_4)\text{alkoxy}$ , and  $r=0-4$ . Preferably,  $r=0$  and  $p=1$ , and more preferably  $Y^1$  and  $Y^2=H$ ,  $r=0$  and  $p=1$ . Exemplary compounds include, without limitation, tris(4-hydroxyphenyl)methane triglycidyl ether, bis(4-hydroxyphenyl)methane diglycidyl ether, and resorcinol diglycidyl ether.

55 In compounds of formula E-II where  $R^{11}=\text{CR}^{13}\text{R}^{14}-\text{Z}-\text{CR}^{13}\text{R}^{14}\text{O}$ ,  $Z$  represents a 5- or 6-membered ring. In such ring structures, the  $\text{CR}^{13}\text{R}^{14}$  groups may be attached at any position, such as at adjacent atoms of the ring or at any other atoms of the ring. Particularly suitable compounds of formula E-II where  $R^{11}=\text{CR}^{13}\text{R}^{14}-\text{Z}-\text{CR}^{13}\text{R}^{14}\text{O}$  are those having the formula

wherein  $Y^1$  and  $Y^2$  are as defined above.

55 Suitable epoxide-containing compounds of formula E-III may be monocyclic, spirocyclic, fused and/or bicyclic rings. Preferred epoxide-containing compounds of formula E-III include 1,2,5,6-diepoxy-cyclooctane, 1,2,6,7-diepoxy-cyclodecane, dicyclopentadiene dioxide, 3,4-epoxytetrahydrothiophene-1,1-dioxide, cyclopentene oxide, cyclohexene oxide, and vinylcyclohexene dioxide.

60 The epoxide-containing compounds useful in the present invention can be obtained from a variety of commercial sources, such as Sigma-Aldrich, or can be prepared using a variety of literature methods known in the art. Mixtures of epoxide-containing compounds may be used.

65 The reaction products of the present invention can be prepared by reacting one or more pyridine compounds described above with one or more epoxide-containing compounds described above. Typically, desired amounts of the pyridine

## 11

compound and epoxide-containing compound are added to a reaction flask, followed by addition of water. The resulting mixture is heated to approximately 75-95° C. for 4 to 6 hours. After an additional 6-12 hours of stirring at room temperature, the resulting reaction product is diluted with water. The reaction product may be used as-is in aqueous solution, may be purified or may be isolated as desired.

In general, the present leveling agents have a number average molecular weight (Mn) of 500 to 10,000, although higher or lower Mn values may be used. Such reaction products may have a weight average molecular weight (Mw) value in the range of 1000 to 50,000, although other Mw values may be used. The Mw values are determined using size exclusion chromatography and a PL Aquagel-OH 8  $\mu$ m, 300 $\times$ 7.5 mm column from Varian, Inc, and polyethylene glycol calibration kit standards from Polymer Standards Service-USA, Inc. Typically, Mw is from 1000 to 20,000, preferably from 1000 to 15,000, and more preferably from Mw is 1500 to 5000. The leveling agents of the present invention may possess any suitable molecular weight polydispersity and work over a wide molecular weight polydispersity range.

Typically, the ratio of the pyridine compound to the epoxide-containing compound is from 0.1:10 to 10:0.1. Preferably, the ratio is from 0.5:5 to 5:0.5 and more preferably from 0.5:1 to 1:0.5. Other suitable ratios of pyridine compound to epoxide-containing compound may be used to prepare the present leveling agents. Mixtures of pyridine compounds may be used in the present invention, as well as mixtures of a pyridine compound with another nitrogen-containing compound.

It will be appreciated by those skilled in the art that a leveling agent of the present invention may also possess functionality capable of acting as a suppressor. Such compounds may be dual-functioning, i.e. they may function as leveling agents and as suppressors.

The present electroplating baths may optionally contain a second leveling agent. Such second leveling agent may be another leveling agent of the present invention, or alternatively, may be any conventional leveling agent. Suitable conventional leveling agents useful in combination with the present leveling agents include, without limitations, those disclosed in U.S. Pat. Nos. 6,610,192 (Step et al.), 7,128,822 (Wang et al.), 7,374,652 (Hayashi et al.), and 6,800,188 (Hagiwara et al.), and in U.S. Pat. App. Pub. Nos. 2011/0220512 (Niazimbetova et al.), 2011/0220513 (Niazimbetova et al.), and 2011/0220514 (Niazimbetova).

The amount of the leveling agent used in the copper electroplating baths will depend upon the particular leveling agents selected, the concentration of the copper ions in the electroplating bath, the particular electrolyte used and its concentration, and the current density applied. In general, the total amount of the leveling agent in the electroplating bath is from 0.01 ppm to 5000 ppm based on the total weight of the plating bath, although greater or lesser amounts may be used. Preferably, the total amount of the leveling agent is from 0.25 to 5000 ppm, more preferably from 0.25 to 1000 ppm and still more preferably from 0.25 to 100 ppm.

Halide ions may optionally be added to the plating bath. Chloride ions are the preferred halide ions. Exemplary chloride ion sources include copper chloride and hydrochloric acid. A wide range of halide ion concentrations may be used in the present invention, such as from 0 to 100 ppm based on the plating bath, and preferably from 10 to 100 ppm. A more preferable amount of halide ion is from 20 to 75 ppm. Such halide ion sources are generally commercially available and may be used without further purification.

## 12

The present plating baths may optionally, and preferably do, contain an accelerator. Any accelerators (also called brightening agents) are suitable for use in the present invention and are well-known to those skilled in the art. Typical accelerators contain one or more sulfur atoms and have a molecular weight of 1000 or less. Accelerator compounds that have sulfide and/or sulfonic acid groups are generally preferred, particularly compounds that include a group of the formula  $R'-S-R-SO_3X$ , where R is optionally substituted alkyl, optionally substituted heteroalkyl, optionally substituted aryl, or optionally substituted heterocyclic; X is a counter ion such as sodium or potassium; and R' is hydrogen or a chemical bond. Typically, the alkyl groups are ( $C_1-C_{16}$ ) alkyl and preferably ( $C_3-C_{12}$ ) alkyl. Heteroalkyl groups typically have one or more heteroatoms, such as nitrogen, sulfur or oxygen, in the alkyl chain. Exemplary aryl groups include phenyl, benzyl, biphenyl and naphthyl. Heterocyclic groups may be aromatic or non-aromatic. Preferred accelerators include: N,N-dimethyl-dithiocarbamic acid-(3-sulfopropyl) ester; 3-mercaptopropylsulfonic acid-(3-sulfopropyl)ester; 3-mercaptopropylsulfonic acid  $Na^+$  salt; carbonic acid-dithio-o-ethylester-s-ester with 3-mercaptopropane sulfonic acid  $K^+$  salt; bis-sulfopropyl disulfide; 3-(benzothiazolyl-s-thio)propyl sulfonic acid  $Na^+$  salt; pyridinium propyl sulfobetaine; 1-sodium-3-mercaptopropane-1-sulfonate; N,N-dimethyl-dithiocarbamic acid-(3-sulfoethyl)ester; 3-mercaptopropylsulfonic acid-(3-sulfoethyl)ester; 3-mercaptopropylsulfonic acid  $Na^+$  salt; carbonic acid-dithio-o-ethylester-s-ester with 3-mercaptopropane sulfonic acid  $K^+$  salt; bis-sulfoethyl disulfide; 3-(benzothiazolyl-s-thio)ethyl sulfonic acid  $Na^+$  salt; pyridinium ethyl sulfobetaine; and 1-sodium-3-mercaptopropane-1-sulfonate.

Accelerators may be used in a variety of amounts. In general, accelerators are used in an amount of at least 0.01 mg/L, based on the bath, preferably at least 0.5 mg/L, and more preferably at least 1 mg/L. The accelerators are present in an amount of from 0.1 to 200 mg/L. The particular amount of accelerator will depend upon the specific application, such as high aspect ratio, through-hole filling, via filling, and wafer plating applications. Preferable amounts of accelerator are at least 0.5 mg/L, and more preferably at least 1 mg/L. A preferable range of accelerator concentrations is from 0.1 to 10 mg/L (ppm). The selection of the accelerator and the amount used is well within the ability of one skilled in the art.

Any compound capable of suppressing the copper plating rate may optionally be used as a suppressor in the present electroplating baths. Exemplary suppressors are polyethers, such as those of the formula  $R-O-(CX_2CX'Y'O)_nR'$  where R and R' are independently chosen from H, ( $C_2-C_{20}$ ) alkyl group and ( $C_6-C_{10}$ ) aryl group; each of X, Y, X' and Y' is independently selected from hydrogen, alkyl such as methyl, ethyl or propyl, aryl such as phenyl, or aralkyl such as benzyl; and n is an integer from 5 to 100,000. Typically, one or more of X, Y, X' and Y' is hydrogen. Preferred suppressors include polypropylene glycol copolymers, polyethylene glycol copolymers, ethylene oxide-propylene oxide ("EO/PO") copolymers and capped EO/PO copolymers, such as butyl alcohol-EO/PO copolymers. Such EO/PO copolymers may be block, alternating or random. Suitable EO/PO copolymers are those sold under the PLURONIC brand name (BASF). Alternate suppressors are EO/PO copolymers derived from an amine core, such as ethylene diamine, and include those available under the TETRONIC brand name (BASF). Typically, suppressors have a weight average molecular weight of 500 to 10,000, and preferably 1000 to 10,000. When such suppressors are used, they are typically present in an amount

of from 1 to 10,000 ppm based on the weight of the bath, and preferably from 5 to 10,000 ppm.

The electroplating baths of the present invention are typically aqueous. Unless otherwise specified, all concentrations of components are in an aqueous system. Particularly suitable compositions useful as electroplating baths in the present invention include a soluble copper salt, an acid electrolyte, an accelerator, a suppressor, halide ion and a reaction product described above as a leveling agent. More preferably, suitable compositions include 10 to 220 g/L of a soluble copper salts as copper metal, 5 to 250 g/L of acid electrolyte, 1 to 50 mg/L of an accelerator, 1 to 10,000 ppm of a suppressor, 10 to 100 ppm of a halide ion, and 0.25 to 5000 ppm of a reaction product described above as a leveling agent.

The electroplating baths of the present invention may be prepared by combining the components in any order. It is preferred that the inorganic components such as source of copper ions, water, electrolyte and optional halide ion source, are first added to the bath vessel followed by the leveling agent and other organic components such as accelerators and suppressors.

The plating baths of the present invention may be used at any suitable temperature, such as from 10 to 65°C. or higher. Preferably, the temperature of the plating baths is from 10 to 35°C. and more preferably from 15 to 30°C. In general, the present copper electroplating baths are agitated during use. Any suitable agitation method may be used with the present invention and such methods are well-known in the art. Suitable agitation methods include, but are not limited to, air sparging, work piece agitation, and impingement.

The present invention is useful for depositing a copper layer on a variety of substrates, particularly those having variously sized apertures. Any substrate upon which copper can be electroplated is useful in the present invention. Such substrates include, but are not limited to, electronic devices such as printed wiring boards, integrated circuit ("IC") substrates including IC packages, lead frames and interconnects. It is preferred that the substrate is a PCB or an IC substrate. In one embodiment, the IC substrate is a wafer used in a dual damascene manufacturing process. Such substrates typically contain a number of features, particularly apertures, having a variety of sizes. Through-holes in a PCB may have a variety of diameters, such as from 50 µm to 2 mm, or greater, in diameter. Such through-holes may vary in depth, such as from 35 µm to 15 mm or greater. PCBs may contain blind vias having a wide variety of sizes, such as up to 200 µm, or greater. The present invention is particularly suitable for filling apertures of varying aspect ratios, such as low aspect ratio vias and high aspect ratio apertures. "Low aspect ratio" means an aspect ratio of from 0.1:1 to 4:1. "High aspect ratio" refers to aspect ratios of greater than 4:1, such as 10:1 or 20:1.

Typically, a substrate is electroplated by contacting it with the plating bath of the present invention. The substrate typically functions as the cathode. The plating bath contains an anode, which may be soluble or insoluble. Potential is typically applied to the cathode. Sufficient current density is applied and plating performed for a period of time sufficient to deposit a copper layer having a desired thickness on the substrate as well as fill blind vias and/or through holes. Suitable current densities, include, but are not limited to, the range of 0.05 to 10 A/dm<sup>2</sup>, although higher and lower current densities may be used. The specific current density depends in part upon the substrate to be plated and the leveling agent selected. Such current density choice is within the abilities of those skilled in the art.

The present invention provides copper layers having a substantially level surface across a substrate surface, even on

substrates having very small features and on substrates having a variety of feature sizes. The copper layers deposited according to the present method have significantly reduced defects, such as nodules, as compared to copper deposits from electroplating baths using conventional leveling agents. Further, the present invention effectively deposits copper in through-holes and blind via holes, that is, the present copper plating baths have very good throwing power. Copper is deposited in apertures according to the present invention without substantially forming voids within the metal deposit. By the term "without substantially forming voids", it is meant that >95% of the plated apertures are void-free. It is preferred that the plated apertures are void-free. Copper is also deposited uniformly in through-holes and in high aspect ratio through-holes with improved throwing power, surface distribution and thermal reliability.

An advantage of the present invention is that substantially level copper deposits are obtained on a PCB. By "substantially level" copper layer is meant that the step height, that is, the difference between areas of dense, very small apertures and areas free of, or substantially free of, apertures is less than 5 µm, and preferably less than 1 µm. A further advantage of the present invention is that a wide range of apertures and aperture sizes may be filled within a single substrate with substantially no suppressed local plating. A further advantage of the present invention is that a substantially planar copper layer may be deposited on a PCB having non-uniformly sized apertures. "Non-uniformly sized apertures" refer to apertures having a variety of sizes in the same PCB.

While the process of the present invention has been generally described with reference to printed circuit board manufacture, it will be appreciated that the present invention may be useful in any electrolytic process where an essentially level or planar copper deposit and filled apertures that are substantially free of voids are desired. Such processes include IC substrates, semiconductor packages and interconnect devices.

#### EXAMPLE 1

In a 100 mL round-bottom, three-neck flask equipped with a condenser and a thermometer, 100 mmol of 4-(dimethylamino)pyridine and 20 mL of DI water were added followed by addition of 63 mmol of 1,4-butanediol diglycidyl ether. The resulting mixture was heated for about 5 hours using an oil bath set to 95°C. and then left to stir at room temperature for additional 8 hours. An amber colored, not-very viscous reaction product was transferred into a 200 mL volumetric flask, rinsed and adjusted with DI water to the 200 mL mark. The reaction product (Reaction Product 1) solution was used without further purification. Analysis of Reaction Product 1 by <sup>1</sup>H NMR (500 MHz, CH<sub>3</sub>OH-d<sub>6</sub>) showed the following peaks, confirming the structure: δ ppm: 8.12-7.80 (m, 2H, 2×H<sub>arom</sub>); 6.98-6.42 (m, 2H, 2×H<sub>arom</sub>); 4.16-3.02 (m, 14.82H (14H×0.63 mole), 4×CH<sub>2</sub>—O, 2×CH—OH, 2×CH<sub>2</sub>—N; 6H, 2×CH<sub>3</sub>—N); 1.72-1.54 (m, 2.52H (4H×0.63 mole), 2×CH<sub>2</sub>).

#### EXAMPLE 2

1,4-Butanediol diglycidyl ether (100 mmol) and 100 mmol of 2-(benzylamino)-pyridine were added at room temperature to a round-bottom reaction flask. Next, 20 mL of DI water were added to the flask. The initially formed white-colored suspension eventually disappeared as the reaction temperature increased and turned into a phase separated mixture. The reaction mixture was heated for 2 hours using an oil bath set to 95°C. After adding 6 mL of 50% sulfuric acid into the

15

reaction flask, the solution became transparent with a light-yellow color. The mixture was heated for an additional 3 hours and left stirring at room temperature for another 8 hours. The resulting amber colored reaction product was transferred into a volumetric flask, rinsed and diluted with 0.5-1% sulfuric acid. The reaction product (Reaction Product 8) solution was used without further purification.

16

## EXAMPLE 3

The reaction products in Table 1 were prepared using the general procedures of Examples 1 or 2. Reaction Products 5 C-1, C-2, and C-3 are comparatives. The UV-absorption of the reaction products was determined in water and the  $\lambda_{max}$  (nm) for the absorbances is also reported in Table 1.

TABLE 1

| Reaction Product | Pyridine-compound (M1) | Epoxide-containing compound (M2) | Molar ratio M1:M2 | $\lambda_{max}$ (nm) |
|------------------|------------------------|----------------------------------|-------------------|----------------------|
| 1                |                        |                                  | 1:0.63            | 206, 266, 288        |
| 2                |                        |                                  | 1:1               | 206, 266, 288        |
| 3                |                        |                                  | 1:0.63            | 242, 315             |
| 4                |                        |                                  | 1:1               | 242, 315             |
| 5                |                        |                                  | 1:1               | 235, 310             |
| 6                |                        |                                  | 1:1               | 205, 269             |
| 7                |                        |                                  | 1:1               | 219, 248, 322        |
| 8                |                        |                                  | 1:1               | 236, 316             |
| 9                |                        |                                  | 1:1               | 336                  |

TABLE 1-continued

| Reaction Product | Pyridine-compound<br>(M1)                                                           | Epoxide-containing compound<br>(M2)                                                  | Molar ratio<br>M1:M2 | $\lambda_{max}$<br>(nm)     |
|------------------|-------------------------------------------------------------------------------------|--------------------------------------------------------------------------------------|----------------------|-----------------------------|
| 10               |    |    | 1:0.63               | 217,<br>236,<br>320,<br>330 |
| 11               |    |    | 1:0.63               | 231,<br>256,<br>301         |
| 12               |    |    | 1:0.63               | Gelled                      |
| 13               |  |  | 1:0.63               | 221,<br>270                 |
| 14               |  |   | 1:1                  | 214,<br>291                 |
| C-1              |  |   | 1:1                  | 238,<br>312                 |
| C-2              |  |   | 1:1                  | 210,<br>275                 |
| C-3              |  |   | 1:1                  | 219,<br>255,<br>331         |

**19**  
EXAMPLE 4

**20**

The general procedures of Examples 1 or 2 are repeated except that the following pyridine-compounds and epoxide-containing monomers are used in the ratios listed in Table 2.

TABLE 2

| Reaction Product | Pyridine-compound (M1) | Epoxide-containing compound (M2) | Monomer 3 (M3) | Molar ratio M1:M2:M3 |
|------------------|------------------------|----------------------------------|----------------|----------------------|
| 15               |                        |                                  |                | 1:0.7:0.3            |
| 16               |                        |                                  |                | 1:1                  |
| 17               |                        |                                  |                | 1:1                  |
| 18               |                        |                                  |                | 1:1                  |
| 19               |                        |                                  |                | 1:1                  |
| 20               |                        |                                  |                | 1:1                  |
| 21               |                        |                                  |                | 1:0.5:0.5            |
| 22               |                        |                                  |                | 1:2:1                |

TABLE 2-continued

| Reaction Product | Pyridine-compound (M1) | Epoxide-containing compound (M2) | Monomer 3 (M3) | Molar ratio M1:M2:M3 |
|------------------|------------------------|----------------------------------|----------------|----------------------|
| 23               |                        |                                  |                | 1:1                  |
|                  |                        | Mw 526                           |                |                      |
| 24               |                        |                                  |                | 1:2:1                |
| 25               |                        |                                  |                | 1:2:1                |
| 26               |                        |                                  |                | 1:2:1                |
|                  |                        | Mw 526                           |                |                      |

## EXAMPLE 5

A copper plating bath was prepared by combining 75 g/L copper as copper sulfate pentahydrate, 240 g/L sulfuric acid, 60 ppm chloride ion, 1 ppm of an accelerator and 1.5 g/L of a suppressor. The accelerator was a disulfide compound having sulfonic acid groups and a molecular weight of <1000. The suppressor was an EO/PO copolymer having a molecular weight of <5,000 and terminal hydroxyl groups. The plating bath also contained 3 mL/L of a stock solution of the reaction product from Example 1.

## EXAMPLE 6

Various copper plating baths were prepared generally according to Example 5, except that each of the reaction products of Examples 2-3 were used in the amount of 0.2-4.0 mL/L, and the amount of accelerator was different where indicated in Table 3.

## EXAMPLE 7

Samples (1.6 mm thick) of a double-sided FR4PCB (5×9.5 cm) having through-holes were plated in a Haring cell using copper plating baths according to Example 4. The samples had 0.25 mm diameter through-holes. The temperature of each bath was 25° C. A current density of 3.24 A/dm<sup>2</sup> (30 A/ft<sup>2</sup>) was applied to the samples for 44 minutes. The copper plated samples were analyzed to determine the throwing power ("TP") of the plating bath, extent of nodule formation, and percent cracking according to the following methods. The amount of the accelerator in each plating bath was 1 ppm. The amount of the leveling agent used in each plating bath and the plating data are shown in Table 3.

Throwing power was calculated by determining the ratio of the average thickness of the metal plated in the center of a

through-hole compared to the average thickness of the metal plated at the surface of the PCB sample and is reported in Table 3 as a percentage.

Nodule formation was determined both by visual inspection and by using the Reddington Tactile Test ("RTT"). Visual inspection showed the presence of nodules while the RTT was used to determine the number of nodules. The RTT employs a person's finger to feel the number of nodules for a given area of the plated surface, which in this example was both sides of the PCB sample (total area of 95 cm<sup>2</sup>).

The percent cracking was determined according to the industry standard procedure, IPC-TM-650-2.6.8. Thermal Stress, Plated-Through Holes, published by IPC (Northbrook, Ill., USA), dated May, 2004, revision E.

Plating bath performance was evaluated by throwing power, number of nodules and cracking. The higher the throwing power (preferably >70%), the lower the number of nodules and the lower the percentage of cracking, the better the plating bath performed. As can be seen from the data, plating bath performance can be easily adjusted by increasing or decreasing the amount of the leveling agent in the plating bath.

TABLE 3

| Reaction Product | ppm | TP (%) | Nodules | Cracking (%) |
|------------------|-----|--------|---------|--------------|
| 1                | 1   | 74     | 0       | 0            |
|                  | 5   | 85     | 2       | 0            |
|                  | 10  | 87     | 3       | 0            |
|                  | 20  | 88     | 5       | 0            |
| 2                | 1   | 83     | 0       | 0            |
|                  | 5   | 82     | 3       | 0            |
|                  | 10  | 66     | 7       | 0            |
|                  | 20  | 78     | 4       | 0            |
| 3                | 1   | 72     | 0       | 0            |
|                  | 5   | 78     | 0       | 0            |

TABLE 3-continued

| Reaction Product | ppm | TP (%) | Nodules | Cracking (%) |    |
|------------------|-----|--------|---------|--------------|----|
| 4                | 10  | 73     | 0       | 0            | 5  |
|                  | 20  | 72     | 0       | 0            |    |
|                  | 1   | 73     | 0       | 0            |    |
|                  | 5   | 74     | 1       | 0            |    |
|                  | 10  | 75     | 2       | 0            |    |
|                  | 20  | 77     | 1       | 0            |    |
|                  | 1   | 81     | 1       | 0            |    |
|                  | 5   | 83     | 8       | 0            |    |
|                  | 10  | 73     | 11      | 0            |    |
|                  | 20  | 72     | 7       | 0            |    |
| 6                | 1   | 84     | 1       | 0            | 15 |
|                  | 5   | 82     | 22      | 0            |    |
|                  | 10  | 81     | 15      | 0            |    |
|                  | 20  | 76     | 25      | 0            |    |
| 7                | 1   | 71     | 1       | 5            | 20 |
|                  | 5   | 69     | 14      | 100          |    |
|                  | 10  | 69     | 10      | 100          |    |
|                  | 20  | 69     | 35      | 100          |    |
| 8                | 1   | 77     | 0       | 0            | 25 |
|                  | 5   | 101    | 0       | 100          |    |
|                  | 10  | 105    | 0       | 100          |    |
|                  | 20  | 87     | 1       | 100          |    |
| 9                | 1   | 66     | 0       | 100          |    |
|                  | 5   | 51     | 2       | 100          |    |
|                  | 10  | 53     | 3       | 100          |    |
| 10               | 0.5 | 77     | 0       | 5            |    |
|                  | 1   | 82     | 0       | 11           |    |
|                  | 5   | 82     | 3       | 19           |    |
|                  | 1*  | 80     | 0       | 15           |    |
|                  | 5*  | 78     | 0       | 0            |    |
|                  | 1** | 74     | 0       | 2            |    |
|                  | 5** | 80     | 0       | 0            |    |
|                  | 0.5 | 71     | 2       | 60           | 30 |
|                  | 1   | 62     | 1       | 75           |    |
|                  | 5   | 61     | 17      | 100          |    |
| 11               | 1*  | 68     | 7       | 69           |    |
|                  | 5*  | 75     | 5       | 98           |    |
|                  | 1** | 73     | 0       | 52           |    |
|                  | 5** | 78     | 6       | 47           |    |
| 13               | 1   | 83     | 0       | 4            | 35 |
|                  | 5   | 85     | 0       | 78           |    |
|                  | 10  | 77     | 0       | 88           |    |
|                  | 20  | 75     | 20      | 100          |    |
| 14               | 1   | 77     | 0       | 0            | 40 |
|                  | 5   | 83     | 2       | 0            |    |
|                  | 10  | 84     | 2       | 0            |    |
|                  | 20  | 92     | 0       | 0            |    |
| C-1              | 1   | 71     | 1       | 0            |    |
|                  | 5   | —      | 0       | 0            |    |
|                  | 10  | 69     | 0       | 0            |    |
|                  | 20  | 61     | 0       | 0            |    |
| C-2              | 1   | 71     | 2       | 100          | 45 |
|                  | 5   | 67     | 35      | 100          |    |
|                  | 10  | 67     | 75      | 100          |    |
|                  | 20  | 67     | 120     | 100          |    |
| C-3              | 1   | 62     | 1       | 9            | 50 |
|                  | 5   | 69     | 7       | 64           |    |
|                  | 10  | 67     | 14      | 100          |    |
|                  | 20  | 67     | 45      | 100          |    |

\*2 ppm of accelerator was used

\*\*3 ppm of accelerator was used

Comparative samples C-1, C-2 and C-3 had lower throwing power, more nodules and more cracking than the corresponding reaction products of the invention, reaction products 5, 6, and 7, respectively. Epichlorohydrin was used as the epoxide-containing compound for samples C-1, C-2 and C-3, where corresponding reaction products 5, 6 and 7 use an epoxide-containing compound that does not contain a leaving group on a carbon alpha to an epoxide group.

What is claimed is:

1. A copper electroplating bath comprising: a source of copper ions; an electrolyte; and a leveling agent; wherein the leveling agent comprises a reaction product of a pyridine compound of the formula (I)

(I)



wherein R<sup>1</sup>, R<sup>3</sup> and R<sup>5</sup> are independently chosen from H, (C<sub>1</sub>-C<sub>6</sub>)alkyl, Cy<sup>1</sup>, R<sup>6</sup>-Cy<sup>1</sup>, NR<sup>7</sup>R<sup>8</sup>, and R<sup>6</sup>-NR<sup>7</sup>R<sup>8</sup>; Cy<sup>1</sup> is a 5- to 6-membered saturated, unsaturated or aromatic ring carbocyclic or heterocyclic ring; R<sup>2</sup> and R<sup>4</sup> are independently chosen from H, (C<sub>1</sub>-C<sub>6</sub>)alkyl, and (C<sub>6</sub>-C<sub>12</sub>)aryl; R<sup>7</sup> and R<sup>8</sup> are independently chosen from H, (C<sub>1</sub>-C<sub>3</sub>)alkyl, phenyl, benzyl and phenethyl; with an epoxide-containing compound; wherein at least one of R<sup>1</sup>, R<sup>3</sup> and R<sup>5</sup> is NR<sup>7</sup>R<sup>8</sup>.

2. The copper electroplating bath of claim 1 wherein the epoxide-containing compound comprises from 1 to 3 epoxide groups.

3. The copper electroplating bath of claim 2 wherein the epoxide-containing compound is chosen from compounds of the formulae



(E-I)



(E-II)



(E-III)

where Y, Y<sup>1</sup> and Y<sup>2</sup> are independently chosen from H and (C<sub>1</sub>-C<sub>4</sub>)alkyl; each Y<sup>3</sup> is independently chosen from H, an epoxy group, and (C<sub>1</sub>-C<sub>6</sub>)alkyl; X=CH<sub>2</sub>X<sup>2</sup> or (C<sub>2</sub>-C<sub>6</sub>) alkenyl; X<sup>1</sup>=H or (C<sub>1</sub>-C<sub>5</sub>)alkyl; X<sup>2</sup>=halogen, O(C<sub>1</sub>-C<sub>3</sub>) alkyl or O(C<sub>1</sub>-C<sub>3</sub>)haloalkyl; A=OR<sup>11</sup> or R<sup>12</sup>; R<sup>11</sup>=((CR<sup>13</sup>R<sup>14</sup>)<sub>m</sub>O)<sub>n</sub>, (aryl-O)<sub>p</sub>, CR<sup>13</sup>R<sup>14</sup>-Z-CR<sup>13</sup>R<sup>14</sup>O or OZ<sup>1</sup>O; R<sup>12</sup>=(CH<sub>2</sub>)<sub>y</sub>; A1 is a (C<sub>5</sub>-C<sub>12</sub>)cycloalkyl ring or a 5- to 6-membered cyclicsulfone ring; Z=a 5- or 6-membered ring; Z<sup>1</sup> is R<sup>15</sup>OArOR<sup>15</sup>, (R<sup>16</sup>O)<sub>a</sub>Ar(OR<sup>16</sup>)<sub>a</sub>, or (R<sup>16</sup>O)<sub>a</sub>Cy<sup>2</sup>(OR<sup>16</sup>)<sub>a</sub>; Z<sup>2</sup>=SO<sub>2</sub> or



Cy<sup>2</sup>=(C<sub>5</sub>-C<sub>12</sub>)cycloalkyl; each R<sup>13</sup> and R<sup>14</sup> are independently chosen from H, CH<sub>3</sub> and OH; each R<sup>15</sup> represents (C<sub>1</sub>-C<sub>8</sub>)alkyl; each R<sup>16</sup> represents a (C<sub>2</sub>-C<sub>6</sub>)alkyleoxy; each a=1-10; m=1-6; n=1-20; p=1-6; q=1-6; r=0-4; t=1-4; v=0-3; and y=0-6; wherein Y<sup>1</sup> and Y<sup>2</sup> may be taken together to form a (C<sub>8</sub>-C<sub>12</sub>)cyclic compound.

25

4. The copper electroplating bath of claim 1 wherein epoxide-containing compound is free of a leaving group on a each carbon alpha to each epoxide group.

5. The copper electroplating bath of claim 4 wherein the leaving group is chosen from chloride, bromide, iodide, tosyl, triflate, sulfonate, mesylate, methosulfate, fluorosulfonate, methyl tosylate, brosylate and nosylate.

6. The copper electroplating bath of claim 1 wherein the pyridine compound is chosen from 2-aminopyridine; 4-aminopyridine; 2-(dimethylamino)pyridine; 4-(dimethylamino)pyridine; 2-(diethylamino)pyridine; 4-(diethylamino)pyridine; 2-(benzylamino)pyridine; and N,N,2-trimethylpyridin-4-amine.

7. A method of depositing copper on a substrate comprising: contacting a substrate to be plated with the copper electroplating bath of claim 1; and applying a current density for a period of time sufficient to deposit a copper layer on the substrate.

8. The method of claim 7 wherein the epoxide-containing compound is chosen from compounds of the formulae



26

where Y, Y<sup>1</sup> and Y<sup>2</sup> are independently chosen from H and (C<sub>1</sub>-C<sub>4</sub>)alkyl; each Y<sup>3</sup> is independently chosen from H, an epoxy group, and (C<sub>1</sub>-C<sub>6</sub>)alkyl; X=CH<sub>2</sub>X<sup>2</sup> or (C<sub>2</sub>-C<sub>6</sub>) alkenyl; X<sup>1</sup>=H or (C<sub>1</sub>-C<sub>5</sub>)alkyl; X<sup>2</sup>=halogen, O(C<sub>1</sub>-C<sub>3</sub>) alkyl or O(C<sub>1</sub>-C<sub>3</sub>)haloalkyl; A=OR<sup>11</sup> or R<sup>12</sup>; R<sup>11</sup>=((CR<sup>13</sup>R<sup>14</sup>)<sub>m</sub>O)<sub>n</sub>, (aryl-O)<sub>p</sub>, CR<sup>13</sup>R<sup>14</sup>—Z—CR<sup>13</sup>R<sup>14</sup>O or OZ<sup>1</sup>O; R<sup>12</sup>=(CH<sub>2</sub>)<sub>y</sub>; A1 is a (C<sub>5</sub>-C<sub>12</sub>)cycloalkyl ring or a 5- to 6-membered cyclicsulfone ring; Z=a 5- or 6-membered ring; Z<sup>1</sup> is R<sup>15</sup>OArOR<sup>15</sup>, (R<sup>16</sup>O)<sub>a</sub>Ar (OR<sup>16</sup>)<sub>a</sub>, or (R<sup>16</sup>O)<sub>a</sub>Cy<sup>2</sup>(OR<sup>16</sup>)<sub>a</sub>; Z<sup>2</sup>=SO<sub>2</sub> or



Cy<sup>2</sup>=(C<sub>5</sub>-C<sub>12</sub>)cycloalkyl; each R<sup>13</sup> and R<sup>14</sup> are independently chosen from H, CH<sub>3</sub> and OH; each R<sup>15</sup> represents (C<sub>1</sub>-C<sub>8</sub>)alkyl; each R<sup>16</sup> represents a (C<sub>2</sub>-C<sub>6</sub>)alkyleneoxy; each a=1-10; m=1-6; n=1-20; p=1-6; q=1-6; r=0-4; t=1-4; v=0-3; and y=0-6; wherein Y<sup>1</sup> and Y<sup>2</sup> may be taken together to form a (C<sub>8</sub>-C<sub>12</sub>)cyclic compound.

9. The method of claim 7 wherein the copper electroplating bath further comprises an accelerator.

10. The copper electroplating bath of claim 1 wherein R<sup>1</sup>, R<sup>3</sup> and R<sup>5</sup> are independently chosen from H, NR<sup>7</sup>R<sup>8</sup>, and R<sup>6</sup>—NR<sup>7</sup>R<sup>8</sup>.

11. The copper electroplating bath of claim 1 wherein R<sup>2</sup> and R<sup>4</sup> are independently chosen from H, methyl, ethyl, propyl, phenyl, benzyl, and phenethyl.

12. The copper electroplating bath of claim 1 wherein Cy<sup>1</sup> is chosen from morpholine, piperidine, and pyrrolidine.

\* \* \* \* \*